# EUROPEAN PATENT SPECIFICATION

(11) **EP 0 560 457 B1**
(45) Date of publication and mention of the grant of the patent: **17.06.1998**
(21) Application number: 93200701.6
(22) Date of filing: 11.03.1993
(51) Int. Cl.: G03C 7/388

(54) **Yellow layer for colour photographic paper**
Gelbschicht für farbphotographisches Papier
Couche jaune pour papier couleur photographique

(30) Priority: 13.03.1992 US 850722
(43) Date of publication of application: 15.09.1993
(73) Proprietor: EASTMAN KODAK COMPANY, Rochester, New York 14650-2201 (US)
(72) Inventor: van Meter, James Philip, c/o Eastman Kodak Company, Rochester, New York 14650-2201 (US); Bagchi, Pranab, c/o Eastman Kodak Company, Rochester, New York 14650-2201 (US); Thomas, Brian, c/o Eastman Kodak Company, Rochester, New York 14650-2201 (US); Rosiek, Thomas Arthur, c/o Eastman Kodak Company, Rochester, New York 14650-2201 (US)
(74) Representative: Nunney, Ronald Frederick Adolphe

(56) References cited:
- EP-A- 0 379 893
- WO-A-90/16011
- FR-A- 2 150 505

## Description

This invention relates to color photographic elements and to a method of preparing the same. More particularly, it relates to photographic elements containing certain yellow coupler dispersions and silver halide having an unexpected increase in photographic activity of the yellow dispersion and also an unexpected increase of the stability of the developed yellow dye to light fade.

Ballasted photographic dye forming couplers are usually incorporated in photographic systems as a colloidal emulsion, usually called a dispersion in the photographic art. The various methods of preparation of photographic coupler dispersions of prior art are illustrated in Figure 1. The coupler is added to a high boiling water immiscible solvent (called a permanent solvent) such as tricresyl phosphate, dibutyl phthalate, etc. Some times a low boiling water miscible solvent (called an auxiliary solvent) such as ethylacetate, propanol, methyl-isobutyl ketone, etc. is also added to promote the solubility of less soluble couplers. The mixture is heated to form a true crystal free solution, called the "coupler solution" as indicated in Figure 1. A second solution of the stabilizing surfactant or surfactants is added to a mixture of gelatin and water and heated to produce a true solution called the "surfactant solution" as indicated in Figure 1. The surfactant used in the "surfactant solution" is usually an anionic surfactant. The "surfactant solution" and the "coupler solution" are then mixed together with mild stirring to form what is known as a "premix". The premix consists of a crude emulsion of the oil phase (i.e., the "coupler solution") in the aqueous phase (i.e., the "surfactant solution"). The crude "dispersion" is composed of droplets of very large particles, of the order of 5-15 µm in diameter and is as such not usable for high quality photographic products. It is necessary to further reduce the particle size by subsequent high shear milling procedures. The crude "premix" is then further milled in an appropriate high shear milling device. If the coupler solution is composed of only "permanent" solvent, then the dispersion is directly usable in photographic product and such dispersions are usually called "direct dispersions". The particle size of such dispersions are generally broadly distributed with an average diameter between 0.1 to 0.3 µm. As direct dispersions do not contain any auxiliary solvents, no water miscible solvent removal is necessary, resulting in a relatively less expensive dispersion preparation process. Such direct dispersions are then appropriate for price sensitive high volume products such as various types of color papers.

When dispersions are prepared with auxiliary solvents an additional step is necessary to remove the water miscible solvent such that it does not evaporate during the cooling operations to cause excessive evaporation load or create an environmentally hazardous situation. Those dispersions that are treated by some type of an evaporation procedure to remove the auxiliary solvent under a controlled condition are called "evaporated" dispersions. Alternatively, the crude premix can be chill set and noodled by extrusion through orifices and washed by cold water to remove the water soluble auxiliary solvent. Dispersions prepared by this process are usually called "washed" dispersions. Washed dispersions are in general more expensive than evaporated dispersions as they may involve up to 50 hours of tedious washing procedures. Both "washed" and evaporated dispersions lead to dispersion droplets that have broad size distribution with mean diameters ranging between 0.1 to 0.3 µm. "Washed" and "evaporated" dispersions are usually suitable for low volume film products.

U.S. Patent 3,860,425, issued June 14, 1975 to Ono et al teaches the use of a mixture of (1) a nonionic surface active agent containing polyoxypropylene units having a molecular weight greater than 500 and polyoxyethylene units, and at a molar ratio of said polyoxyethylene units to the polyoxypropylene units ranging from 0.1 to 0.6 and (2) an anionic surface active agent having an -OSO₃M group or an -SO₃M group, wherein M represents a monovalent cation, and a hydrophobic group in the preparation of a milled dispersion of oleophilic materials, for photographic use. Such dispersions have particle diameters between 0.67 to 0.19 µm. Between about 0.05 to about 0.10 gram of the anionic surfactant and between about 0.02 gram to about 0.10 gram of the nonionic surfactant per gram of the oleophilic dispersed phase of the coupler are used.

U.S. Patent 5,013,640, issued May 7, 1991 to Bagchi et al discloses the use of block oligomeric surfactants comprising hydrophobic polyoxyethylene block (A) and hydrophilic polyoxypropylene block (B) joined in the manner of A-B-A, B-A-B, A-B, (A-B)ₙ≅G≅(B-A)ₙ, a (B-A)≅G≅(A-B)ₙ, where G is a connector organic moiety and n is between 1 and 3, as melt addenda to reduce viscosity of a microprecipitated dispersion melt in gelatin. The said microprecipitated dispersion being preprecipitated as a slurry in water before gelatin addition using preferably an anionic surfactant. The particle size of the microprecipitated dispersions have diameters between 0.01 to 0.05 µm.

EP-A-379893 discloses the use of polypropylene oxides having an OH-content of 1-3 wt% as oil formers for use in preparing dispersions of nondiffusible color providing compounds such as color couplers. The oil formers are disclosed as being prepared by reacting water or an alcohol with propylene oxide so as to attain a statistic distribution of the molecular weight of the polypropylene oxide across the entire molecule (page 2, lines 48-53).

In cost sensitive high volume products, such as Ektacolor® Paper or Eastman Color Print®, it is desirable to increase the dye yield of a coupler, as in such a case, it requires less coupler and/or silver, which translates to cost reduction. Further, cyan, magenta and yellow dyes that create photographic images, fade with time when exposed to various ambient lighting conditions such as sunlight, incandescent light or fluorescent light. Most damage is usually done by UV-radiation that may be present in any lighting source. It is therefore desirable to make photographic products, especially photographic paper that is used to display images of both personal and commercial scenes, as stable as possible to fade. There are various means of achieving improved dye stability. One way is to produce couplers that form dye with increased dye stability. Since products such as Ektacolor® Paper or Eastman Color Print® are high volume products that are highly price sensitive, it is not always commercially feasible to replace an existing coupler with settled down cost with a new coupler. Photographic papers contain a layer comprising a UV-absorbing compound dispersed in protective layers to absorb the damaging UV-radiation and prevent it from reaching the image dyes. Usually such UV-absorbing compounds have a slight yellow coloration, which when applied in large enough quantities cause the white areas of paper to appear yellow, which is highly undesirable. Therefore, there is a limit to the extent that such UV-absorptive materials can be applied in a photographic product such as paper. U.S. Patent 4,656,125 issued April 7, 1987, to Rinner et al discloses that dye stability can be achieved by the addition of stabilizer compounds to the coupler dispersions. A need to enhance the activity of photographic couplers and enhance the stability of image dyes from fade is desired.

In photographic paper where the image resides on a reflective support light passes through the photographic layers twice for the visualization of the image. In transparency display products such as Duratrans® light passes through the image only once. Therefore, to produce enough visual density the couplers and the silver halide emulsions are coated at about 70% higher levels on a transparent support. In such case, where the component loading is very high, the bottom yellow layer develops up much more slowly compared to the top cyan and the magenta layers. This requires the use of a longer development time. Therefore, a more active bottom yellow layer in such products with faster development rates will provide a much improved product with shorter development time. Therefore, there is need for the invention of a more active yellow dispersion melt.

An object of this invention is to provide more active, (one yielding more dye-density per unit lay down) yellow couplers, dispersed by conventional milling procedures by the simple addition of polyoxyalkylene compounds to the dispersion melt just prior to coating of a photographic product.

Another object of the invention is to provide more light-stable yellow dye-forming coupler dispersion melts for quality improvement of photographic products such as color papers and color display materials.

Another objective of this invention is to provide a multilayer photographic package, where the bottom slow-developing yellow layer is more active.

It has been discovered, quite unexpectedly, that when polymeric, polyoxyalkylene surface active compounds are added to conventional dispersions of pivalylacetanilide (PAA)-yellow couplers, such dispersions in a coated silver halide photographic element produce substantially higher dye yield compared to the conventional dispersion without any additive. Further, the yellow dye formed from such dispersions containing the addenda of this invention are substantially more light stable compared to dispersions that do not contain such addenda.

According to the present invention therefore there is provided a color photographic recording element comprising at least one blue-sensitive photographic silver halide emulsion layer comprising dispersed particles having an average diameter of 0.1 to 0.3 µm and being other than microprecipitated particles, and comprising a yellow image-dye forming pivalylacetanilide coupler, characterized in that the emulsion layer further comprises from about 0.1 to about 0.6 gram of a polyoxyalkylene polymer, per gram of the yellow coupler, wherein the polyoxyalkylene polymer is a non-aromatic polyoxyethylene-polyoxypropylene block co-polymer having at least two terminal hydroxy groups.

Preferably the polyoxyalkylene polymer is present in the amount of from about 0.1 to about 0.3 gram per gram of yellow coupler.

In a preferred embodiment the structure of PAA class yellow couplers to which this invention applies is as follows: where X = H or a coupling off group, and in particular wherein X is -H, -Cl, -OCOR¹ -SAr, SO₂R¹, -OSO₂R¹, where R1 is alkyl; R2 is alkyl, optionally substituted arylsulfonyl, alkoxycarbonyl,
alkylsulfonamido, or carboxyl; R³ is hydrogen or alkylsulfonamino; Ar is aryl; Z is any organic moiety to complete the ring, and Y is a ballasting group.

When R2 is arylsulfonyl, it may be substituted, for example, with PhOCH₂PhOH or NHCH₂CH₂OH.

Ballasting groups usually comprise one or more 5 to 25 carbon atom containing organic moiety whose function is to immobilize the coupler and the formed image dye during photographic development by imparting poor water diffusibility to the coupler compound. Kodachrome® type couplers, however, are unballasted and therefore are soluble in developer solutions. Such couplers are usually incorporated in the developer solutions. Fisher couplers usually contain a solubilizing -SO₃ ⁻ group to impart base solubilizing characteristics to the coupler molecule. In polymeric couplers, the ballast is the polymer backbone which may also be gelatin. In some polymeric couplers the bonding to the ballasting polymeric backbone is achieved through the coupling off group rendering the formed dye more mobile and transferable by diffusion or by thermal evaporation after photographic development. A broad description of such coupler compounds can be found in "The Theory of the Photographic Process", 4th Edition, McMillan, New York, 1977 by T.H. James. Typical ballast group -Y- are extensively described in US 3,770,446 (1973), US 3,265,506 (1966) etc. and are hereby incorporated herein by reference. Broad groups of various ballast groups that can be used are disclosed in US patents 2,875,057; 2,407,210; 2,298,443; 3,048,194; 4,022,620; 4,443,536 and 3,447,928, which are also included herein by reference.

The invention is carried out by adding required amounts of the polymeric polyoxyalkylene surface active compound and preferably a surface active compound comprising at least a polyoxypropylene (POP) block and a polyethylene (POE) block to the dispersion melts, prepared by conventional milling procedure prior to coating the film product.

Thus according to another aspect of the present invention there is provided a a method of preparing a blue sensitive layer in a silver halide photographic light sensitive element which comprises forming a dispersion of a yellow image dye-forming coupler having particles with an average diameter of 0.1 to 0.3 µm, in a hydrophilic colloid, mixing the dispersion with a silver halide emulsion and applying the resulting composition to form a layer, characterized in that the yellow coupler is a pivalylacetanilide coupler and the method further comprises the step of adding a polyoxyalkylene polymer to the dispersion or the emulsion in the amount of from about 0.1 to 0.6 gram per gram of yellow coupler in the dispersion prior to forming the layer.

Drawings are included to illustrate the advantages of this invention. Briefly, the drawings are:
Fig. 1 is a diagrammatic flow chart illustrating prior art procedures for the preparation of conventional milled dispersions.
Fig. 2 is a graph of fresh sensitometric curves comparing several preparations in accordance with the invention to a control.
Fig. 3 is a graph of dye density vs. silver coverage comparing several preparations in accordance with the invention to a control.
Fig. 4 is a graph of fresh sensitometric curves comparing a preparation in accordance with the invention to a control.

The methods of preparation of conventional milled dispersions of photographic dye-forming couplers have been extensively described earlier. In the method and composition of this invention, the surfactant used to prepare the surfactant solution of Fig. 1 is any surfactant that will aid the formation of stable dispersions of particles.

Such surfactants for the preparation of the dispersion can be anionic and are in general defined as follows:

### Class - A: Anionic Dispersion Surfactants:

The anionic dispersion surfactants of this invention comprise a 6 to 25 carbon atom hydrophobic moiety made up of either aliphatic, aromatic or of both types of hydrocarbons, or fluorocarbon groups terminated by single or multiple anionic charges arising from -COO⁻, -SO₃⁻ or -OSO₃⁻ groups or a combination thereof.

Typical examples of such "Class-A Anionic Dispersion Surfactants" are as follow:

DS-A8 ―do― R= ―CH₂ ―CH(CH₂CH₃)C₃H₇

Such surfactants for the preparation of the dispersions can also be polyether surfactants definable as follows:

### Class -B: Polyether Dispersion Surfactants:

The polyether dispersion surfactants of this invention comprise a 6 to 25 carbon atom hydrophobic moiety made up of either aliphatic, aromatic or of both types of hydrocarbon or fluorocarbon groups and at least 2 oxyethylene and/or glycidyl ether groups that may or may not be terminated with a single or multiple negative change arising from -COO⁻, -0SO₃ ⁻,or -OSO₄ ⁻ groups or a combination thereof.

Typical examples of such "Class-B Polyether Dispersion Surfactants" are as follows:

DS-B5 n-C₁₂H₂₅ ―O―(CH₂ -CH₂ -O)₂₃-OH (Trycol 5964, Henkel)

Such surfactants for the preparation of the dispersion can also be sugar surfactants defined as follows:

### Class -C: Sugar Dispersion Surfactants:

The sugar dispersion surfactants of this invention are characterized by having one to three hydrophobic tails, each tail containing from about 6 to 25 carbon atoms comprising either aliphatic, aromatic or a combination of both types of hydrocarbon or fluorocarbon groups and also having one or more attached hydrophilic mono- or oligosacharidic hydrophilic chains that may or may not be terminated by single or multiple anionic charges arising from -COO⁻, -OSO⁻ ₃ or -SO⁻ ₃ groups or a combination thereof.

Typical examples of such "Class -C Sugar Dispersion Surfactants" are as follows:

The dispersion surfactant or surfactants can be used by themselves or as any combination of mixtures of different classes or different individual surfactants at a level performing between about 0.03g to about 0.lg of total surfactant, as a single surfactant or in combination for the preparation of the dispersion per g of the coupler to be dispersed. The preferred surfactant is Alkanol-XC (DS-A11).

Other surfactants of class-A, B or C set forth in "McCutcheon's", Vol. 1, "Emulsifiers and Detergents", International Edition and North American Edition, McCutcheon's Division of the Manufacturing Confectioner Publishing Co., N.J. (1991), incorporated herein by reference, may be used.

The couplers of this invention are yellow-dye forming pivalylacetanilide (PAA) couplers of general structure as indicated earlier. Specific examples of such class of couplers are as follows:

Suitable surface active polyoxyalkylene polymers and preferably block polymeric compounds containing polyoxyethylene and polyoxypropylene blocks or block polymers with multiple polyoxyethylene-polyoxypropylene blocks connected together by an organic moiety that impart high activity and high dye-stability when added to a silver halide gelatino coating melt containing conventionally predispersed PAA couplers of this invention, are given to Table I.

Other polyethylene/polypropylene block containing compounds disclosed in McCutcheon's, Vol 1, "Emulsifiers and Detergents" mention previously may be employed in this invention.

The block polymeric addenda of this invention is added to a coating melt to the extent of 0.1 to 0.6g per gram of the PAA coupler of this invention. The preferred amount is between 0.1 to 0.3g of the block polymeric compound per gram of the PAA coupler. The preferred block polymeric materials of this invention are (P-1) through (P-6). Particularly preferred are polyoxyalkylene polymers of the formula: or where a has a value of 5 to 500 and, b has a value of 5 to 500. Most preferred is Pluronic L44 which has the following structure.

This invention is very specific to couplers of the PAA class. The addition of the surface active materials of this invention produce no activity advantage or dye stability advantage to other couplers. The noninventive coupler combinations with the surface active addenda of this invention exemplified hereinafter are as follows:

Not all nonionic surface active materials show this unique simultaneous effect of increased activity and added dye stability. The noninventive, nonionic surfactant used in this example is the alkyl polyglycoside (APG-225), which has the following structure.

### Examples

The following examples are intended to be illustrative and not exhaustive of the invention. Parts and percentages are by weight unless otherwise specified.

Coating laydowns are given in "mg/ft²". Multiplication of these numbers by 10.7 will convert them to "mg/m²".

### Examples 1 - 7: Dispersions Utilized

Conventional dispersions of the compounds indicated in Table II were prepared according to the description given earlier by the direct method for the reduction to practice of this invention. The various solvents used in preparing these dispersions are as follows:

Dye stabilizers and associated scavengers used in preparation of these dispersions are as follows:

The UV-absorbing compounds used in the layers over the sensitized layers are as follows:

### Examples 8-15: Photographic Coatings and Evaluation Using PAA-Coupler (CY-1)

The coating format for testing these PAA-yellow couplers, from the base up, is as follows:
Base: Titanium dioxide loaded polyethylene resin coated photographic paper stock.
Blue Sensitized Layer: Blue sensitized cubic silver chloride emulsion with up to about 1% surface iodide having an average cubic edge length of about 0.6 microns at 30 mg/ft². Yellow dye-forming coupler (CY-1) at 100 mg/ft² dispersion of Example 1, gelatin at 115 mg/ft², added surfactant (inventive and noninventive at 0, 0.2, and 0.6 g of coupler (CY-1).
UV-Absorbing Layer: UV-absorbing compounds (UV-2) and (UV-1) in dispersion of Example 7 at 80 mg/ft², gelatin at 121 mg/ft².
Overcoat: 125 mg/ft² of gelatin and gelatin hardener bis(vinylsulfonylmethyl)ether (BVSME) at the level of 2% based upon total gel in the packet.

In all layers the spreading agent Olin 10G (Dixie Corporation) was used at a level of 0.3% of the melt volume of each layer.

The coatings were exposed to white light through a gray wedge chart and then processed by the Kodak RA-4 process (Kodak is a trademark of the Eastman Kodak Co.). The resultant image was then read by a color densitometer and the results are summarized in Table III. It is observed in Table III, that in the inventive coatings where the material of this invention, L44, was spiked in at levels of 0.2 and 0.6g per gram of the coupler, large increases in Dmax and contrast (gradient) are shown, with other photographic parameters such as Dmin, and speed remaining the same. Such large boost in limiting reflection density levels indicate large increases in dye density yield. Extraction of the dye from the coatings and determination of their yield with a known extinction coefficient of the dye for the two invention Examples 9 and 10 are also shown in Table III in comparison with the control Example 8. It is seen that in Example 9 there is about a 46% and in Example 10 about 60% increased dye yield. The addition of L44 increased the dye yield for coupler (CY-1). APG 225 which is also a nonionic amphiphile did not show any increase in dye density (Table III). The actual sensitometric curves of the control Example 8 and the invention Examples 9 and 10 are also shown in Fig. 2, where it is seen that the spiking of L44 produces a very large boost in the Dmax of the coating of PAA coupler (CY-1). It is also seen that the boost in activity is nonlinear. That is, the major increase occurs up to a level of 0.2 g per g of coupler (CY-1) and beyond this amount the effect levels off. Fig. 3 shows plots of the dye density yield vs silver formed in the step wedge image as measured by x-ray fluorescence, after fixing out the Ag halide following the color development step. The invention examples show larger dye density for the same amount of silver developed in comparison to the control coatings.

Another advantage of this invention, is high dye stability of the formed dye image. This was demonstrated by exposing the images for 2 and 4 weeks to high intensity (50 K Lux) light balanced to the color temperature of sunshine under ambient humidity and temperature conditions. The density losses measured from a density of 1.7 are also listed in Table III. It is observed that in the inventive Examples 9 and 10 where L44 was present dye density losses were considerably smaller compared to the control Example 8 and the noninventive Example 11 which contained the noninventive material APG 224. It is observed that control Example 8 did not contain any L44.

In a second coating set, similar spiking experiments were done with other polyalkylene compounds such as polyethylene oxide (MW 1500), and polyalkylene block oligomers such as Pluronic P-75 and Tetronic T-304. Table IV shows that these compounds in accordance with this invention with PAA coupler (CY-1) produced increase Dmax, contrast and stability to dye fade under exposure of 50 K Lux sunshine temperature balanced illumination. From the extent of the effects observed, it appears that the block polyalkylene polymers are preferred over the polyoxyethylene compound examined.

### Examples 16 - 17: Photographic Coatings and Evaluation Using PAA-Coupler (CY-2)

The coating format for testing yellow coupler (CY-2), from the base up, is as follows:
Base: Resin coated paper stock as described in Examples 8 - 15.
Blue Sensitized Layer: Blue sensitized cubic silver chloride emulsion with up to about 1% surface bromide having an average cube edge length of about 0.6 micron at 24 mg/ft², yellow dye forming coupler (CY-2) at 50 mg/ft² (dispersion of Example 2), gelatin at 115 mg/ft², added surfactant L-44 0 and 0.2g per g f coupler (CY-2).
UV-Absorbing Layer: UV-absorbing compounds (UV-2) and (UV-1) in dispersion of Example 7 at 80 mg/ft², gelatin at 121 mg/ft².
Overcoat: 125 mg/ft² of gelatin and gelatin hardener bis(vinylsulfonylmethyl)ether (BVSME) at the level of 2% based upon total gel in the packet.

In all layers the spreading agent Olin 10G was used at a level of 0.3% of the melt volume of each layer.

The coatings were exposed and processed in the same manner as indicated earlier. Results are tabulated in Table V. It clearly shows that coupler (CY-2) shows enhancement of Dmax, gradient and dye stability with the addition of the combination agent of this invention, L44, in the layer where the coupler resides. The fresh sensitometry of the coatings of Examples 16 and 17 are shown in Fig. 4.

### Example 18: Photographic Coating and Evaluation Using Thiopyrazolone Magenta Coupler (C-1) (Comparative)

The coating format for testing magenta coupler (C-1), from base up, is as follows:
Base: Resin coated paper stock as described in Examples 8 - 15.
Green Sensitized Layer: Green sensitized cubic silver chloride emulsion with up to about 1% surface bromide having an average cubic edge length of about 0.3 micron at 17 mg/ft², magenta dye-forming coupler (C-1) at 32 mg/ft², with associated image stabilizers as indicated in the dispersion of Example 4, gelatin at 115 mg/ft², added surfactant Pluronic L44 at 0, 20 and 60 mg/ft².
Overcoat: 125 mg/ft² of gelatin and gelatin and hardener BVSME at levels of 2% based upon total gel in the packet.

In all layers the spreading agent Olin 10G was used at a level of 0.3% of the melt volume of each layer.

The coatings were exposed and processed in the same manner as indicated earlier. Sensitometric data, both fresh and after exposure to prolonged high intensity illumination, did not show any activity or dye stability advantages.

### Example 19: Photographic Coatings and Evaluation Using Pyrazolone Magenta Coupler (C-2) (Comparative)

The coating format for testing magenta coupler (C-2), from base up, is as follows:
Base: Resin coated paper stock as described in Examples 8 - 15.
Green Sensitized Layer: Green sensitized cubic silver chloride emulsion with up to 1% surface bromide having an average cubic edge length of about 0.3 micron at 26.5 mg/ft², magenta dye-forming coupler (C-2) at 41.5 mg/ft², with associated image stabilizers as indicated in dispersion of Example 3, gelatin at 115 mg/ft², added surfactant Pluronic L44 at 0, 20 and 60 mg/ft².
UV-Absorbing Layer: UV-absorbing compounds (UV-2) and (UV-1) in dispersion of Example 7 at 80 mg/ft², gelatin at 121 mg/ft².
Overcoat: 125 mg/ft² of gelatin and hardener BVSME at levels of 2% based upon total gel in the packet.

In all layers the spreading agent Olin 10G was used at a level of 0.3% of the melt volume of each layer.

The coatings were exposed and processed in the same manner as indicated earlier. Sensitometric data, both fresh and after exposure to prolonged high intensity illumination, did not show any activity or dye stability advantages.

### Example 20: Photographic Coatings and Evaluation Using Phenolic Cyan Coupler (C-3) (Comparative)

The coating format for testing cyan coupler (C-3), from base up, is as follows:
Base: Resin coated paper stock as described in Examples 8 - 15.
Red Sensitized Layer: Red sensitized cubic silver chloride emulsion with up to 1% surface bromide having an average cubic edge length of about 0.38 micron at 16.7 mg/ft². Cyan dye-forming coupler (C-3) at 39.3 mg/ft² as indicated in dispersion of Example 5. Gelatin at 115 mg/ft², added surfactant Pluronic L44 at 0, 20, and 60 mg/ft².
UV-Absorbing Layer: UV-absorbing compounds (UV-2) and (UV-1) in dispersion of Example 7 at 40 mg/ft², gelatin at 61 mg/ft².
Overcoat: 126 mg/ft² of gelatin and hardener BVSME at levels of 2% based upon total gel in the packet.

In all layers the spreading agent Olin 10G was used at a level of 0.3% of the melt volume of each layer.

The coatings were exposed and processed in the same manner as indicated earlier. Sensitometric data, both fresh and after exposure to prolonged high intensity illumination did not show any activity or dye stability advantages.

### Example 21: Photographic Coatings and Evaluation Using Phenolic Cyan Coupler (C-4) (Comparative)

The coating format for testing cyan coupler (C-4), from base up, is as follows:
Base: Resin coated paper stock as described in Examples 8 - 15.
Red Sensitive Layer: Red sensitive cubic chloride emulsion with up to 10% surface bromide having average cubic edge length of about 0.38 micron at 20 mg/ft², cyan dye-forming coupler (C-4) at 40 mg/ft² as indicated in dispersion of Example 6, gelatin at 100 mg/ft², addenda Pluronic L44 at 0, 20 and 60 mg/ft².
UV-Absorbing Layer: UV-absorbing compounds (UV-2) and (UV-1) in dispersion of Example 7 at 40 mg/ft², gelatin at 61 mg/ft².
Overcoat: 126 mg/ft² of gelatin and hardener BVSME at levels of 2% based upon total gel in the packet.

In all layers the spreading Olin 10G was used at a level of 0.3% of the melt volume of each layer.

The coatings were exposed and processed in the same manner as indicated earlier. Sensitometric data, both fresh and after exposure to prolonged high intensity illumination, did not show any activity or dye stability advantages.

A typical full multilayer photographic element in accordance with this invention has the following configuration:

| | |
|---|---|
| (Numbers indicate coverage in mg per square ft.) (Numbers within " " indicate same in mg per square meter) | |

| LAYER 7 | |
|---|---|
| Overcoat: | |
| 125.0 | Gelatin; "1336" |
| 2.0 | (ST-3) (Conventional Scavenger Dispersed in Solvent); "21" |

| LAYER 6 | |
|---|---|
| UV Protection Layer: | |
| 61.0 | Gelatin; "653" |
| 34.3 | Tinuvin 328 (Co-dispersed) Ultraviolet light absorber; "364" |
| 5.7 | Tinuvin 326 (Co-dispersed) Ultraviolet light absorber; "60" |
| 4.0 | (ST-3) (Co-dispersed in Solvent); "43" |

| LAYER 5 | |
|---|---|
| Red Layer: | |
| 115.0 | Gelatin; "1230" |
| 39.3 | (C-3) (Cyan Cplr. Co-dispersed in Solv.); "420" |
| 0.5 | (ST-3) (Scavenger Co-dispersed in Solvent); "5" |
| 16.7 | AgCl (In Red Sensitized AgCl Emulsion); "179" |

| LAYER 4 | |
|---|---|
| UV Protection Layer: | |
| 61.0 | Gelatin; "653" |
| 34.3 | Tinuvin 328 (Co-dispersed); "364" |
| 5.7 | Tinuvin 326 (Co-dispersed); "60" |
| 4.0 | (ST-3) (Co-dispersed in Solvent); "43" |

| LAYER 3 | |
|---|---|
| Green Layer: | |
| 115.0 | Gelatin; "1230" |
| 41.5 | (C-2) (Magenta Coupler Co-dispersed in Solvent); "444" |
| 18.2 | (ST-1) (Stabilizer Co-dispersed in Solvent); "195" |
| 3.4 | (ST-3) (Scavenger Co-dispersed in Solvent); "37" |
| 24.5 | AgCl (In Green Sensitized AgCl Emulsion); "262" |

| LAYER 2 | |
|---|---|
| Inter Layer: | |
| 70.0 | Gelatin; "749" |
| 9.0 | (ST-3) (Scavenger Dispersed in Solvent); "96" |

| LAYER 1 | |
|---|---|
| Blue Layer: | |
| 140.0 | Gelatin; "1498" |
| 100.0 | (CY-1) (Yellow Coupler Dispersed in Solv.); "1070" |
| 30.0 | AgCl (In Blue Sensitized AgCl Emulsion); "321" |
| 20.0 | Pluronic L-44 "214" |
| Resin Coat | Titanox Dispersed in Polyethylene |
| Support | Paper |
| Resin Coat | Polyethylene |

The invention has been described in detail with particular reference to preferred embodiments thereof, but it will be understood that variations and modifications can be effected within the spirit and scope of the invention.

## Claims

1. A color photographic recording element comprising at least one blue-sensitive photographic silver halide emulsion layer comprising dispersed particles having an average diameter of 0.1 to 0.3 µm, and being other than microprecipitated particles, and comprising a yellow image-dye forming pivalylacetanilide coupler, characterized in that the emulsion layer further comprises from about 0.1 to about 0.6 gram of a polyoxyalkylene polymer, per gram of the yellow coupler, wherein the polyoxyalkylene polymer is a non-aromatic polyoxyethylene-polyoxypropylene block co-polymer having at least two terminal hydroxy groups.

2. The color photographic recording element as claimed in claim 1 wherein the polyoxyalkylene polymer is present in the amount of from about 0.1 to about 0.3 gram per gram of yellow coupler.

3. The color photographic recording element as claimed in claim 1 wherein the yellow image dye forming coupler dispersion contains a coupler solvent.

4. The color photographic recording element as claimed in claim 1 wherein the polyoxyalkylene polymer is where a has a value of 5 to 500 and b has a value of 5 to 500.

5. The color photographic recording element as claimed in any one of the preceding claims wherein the yellow coupler is of the formula: where X is hydrogen or a coupling-off group and Y is a ballasting group.

6. The color photographic recording element as claimed in claim 5 wherein X is -H, -Cl,-OCOR¹,-SAr, -SO₂R¹, -OSO₂R¹, where R¹ is alkyl; R² is alkyl, optionally substituted arylsulfonyl, alkoxycarbonyl, alkylsulfonamido, or carboxyl; R³ is hydrogen or alkylsulfonamido; Ar is aryl; and Z is any organic moiety to complete the ring.

7. A method of preparing a blue sensitive layer in a silver halide photographic light sensitive element which comprises forming a dispersion of a yellow image dye-forming coupler in a hydrophilic colloid, mixing the dispersion with a silver halide emulsion and applying the resulting composition to form a layer, characterized in that the yellow coupler is a pivalylacetanilide coupler and the method further comprises the step of adding a polyoxyalkylene polymer to the dispersion or the emulsion in the amount of from about 0.1 to about 0.6 gram per gram of yellow coupler in the dispersion prior to forming the layer.

8. The method as claimed in claim 7 wherein the polyoxyalkylene polymer is a polyoxyethylene-polyoxypropylene block polymer.

9. The method as claimed in either of claims 7 or 8 wherein the yellow coupler is as defined in either of claims 5 and 6.

## Patentansprüche

1. Farbphotographisches Aufzeichnungselement mit mindestens einer blau-empfindlichen photographischen Silberhalogenidemulsionsschicht mit dispergierten Teilchen mit einem mittleren Durchmesser von 0,1 bis 0,3 µm, wobei es sich bei diesen Teilchen um andere Teilchen handelt als um durch Mikroausfällung erhaltene Teilchen, und mit einem einen gelben Bildfarbstoff liefernden Pivalylacetanilidkuppler, dadurch gekennzeichnet, daß die Emulsionsschicht weiterhin etwa 0,1 bis etwa 0,6 g eines Polyoxyalkylenpolymeren pro g gelbem Kuppler enthält, wobei das Polyoxyalkylenpolymer ein nicht-aromatisches Polyoxyethylen-polyoxypropylen-Blockcopolymer mit mindestens zwei terminalen Hydroxygruppen ist.

2. Farbphotographisches Aufzeichnungselement nach Anspruch 1, in dem das Polyoxyalkylenpolymer in einer Menge von etwa 0,1 bis etwa 0,3 g pro g gelbem Kuppler vorliegt.

3. Farbphotographisches Aufzeichnungselement nach Anspruch 1, in dem die den gelben Bildfarbstoff erzeugende Kupplerdispersion ein Kupplerlösungsmittel enthält.

4. Farbphotographisches Aufzeichnungselement nach Anspruch 1, in dem das Polyoxyalkylenpolymer besteht aus: oder worin a einen Wert von 5 bis 500 und b einen Wert von 5 bis 500 hat.

5. Farbphotographisches Aufzeichnungselement nach einem der vorstehenden Ansprüche, in dem der gelbe Kuppler der Formel entspricht: worin X für Wasserstoff steht oder eine abkuppelnde Gruppe und Y eine Ballastgruppe ist.

6. Farbphotographisches Aufzeichnungselement nach Anspruch 5, in dem X steht für -H, -Cl, -OCOR¹, -SAr, -SO₂R¹, -OSO₂R¹, worin R¹ steht für Alkyl; R² steht für Alkyl, gegebenenfalls substituiertes Arylsulfonyl, Alkoxycarbonyl, Alkylsulfonamido oder Carboxyl; R³ steht für Wasserstoff oder Alkylsulfonamido; Ar steht für Aryl; und Z ist ein beliebiger organischer Rest, um den Ring zu vervollständigen.

7. Verfahren zur Herstellung einer blau-empfindlichen Schicht in einem lichtempfindlichen photographischen Silberhalogenidelement, das umfaßt die Herstellung einer Dispersion eines einen gelben Bildfarbstoff erzeugenden Kupplers in einem hydrophilen Kolloid, das Vermischen der Dispersion mit einer Silberhalogenidemulsion und die Verarbeitung der erhaltenen Zusammensetzung unter Erzeugung einer Schicht, dadurch gekennzeichnet, daß der gelbe Kuppler ein Pivalylacetanilidkuppler ist und daß das Verfahren weiterhin umfaßt die Stufe der Zugabe eines Polyoxyalkylenpolymeren zur Dispersion oder Emulsion in der Menge von etwa 0,1 bis etwa 0,6 g pro g gelbem Kuppler in der Dispersion, bevor die Schicht erzeugt wird.

8. Verfahren nach Anspruch 7, in dem das Polyoxyalkylenpolymer ein Polyoxyethylen-polyoxypropylen-Blockpolymer ist.

9. Verfahren nach einem der Ansprüche 7 oder 8, in dem der gelbe Kuppler ein Kuppler nach einem der Ansprüche 5 und 6 ist.

## Revendications

1. Elément d'enregistrement photographique couleur comprenant au moins une couche d'émulsion photographique aux halogénures d'argent sensible au bleu comprenant des particules dispersées ayant un diamètre moyen compris entre 0,1 et 0,3 µm, autres que des particules microprécipitées, et comprenant un coupleur pivalylacétanilide formateur de colorant d'image jaune, caractérisé en ce que la couche d'émulsion comprend aussi 0,1 à 0,6 gramme environ d'un polymère de polyoxyalkylène par gramme de coupleur jaune, dans lequel le polymère de polyoxyalkylène est un copolymère séquence non aromatique de polyoxyéthylène et de polyoxypropylène ayant au moins deux groupes hydroxy terminaux.

2. Elément d'enregistrement photographique couleur selon la revendication 1, dans lequel le polymère de polyoxyalkylène est présent à une concentration comprise entre 0,1 et 0,3 gramme environ par gramme de coupleur jaune.

3. Elément d'enregistrement photographique couleur selon la revendication 1, dans lequel la dispersion de coupleur formateur de colorant d'image jaune contient un solvant de coupleur.

4. Elément d'enregistrement photographique couleur selon la revendication 1, dans lequel le polymère de polyoxyalkylène est où la valeur de a est comprise entre 5 et 500 et la valeur de b est comprise entre 5 et 500.

5. Elément d'enregistrement photographique couleur selon l'une quelconque des revendications précédentes, dans lequel le coupleur jaune répond à la formule : où X est un hydrogène ou un groupe qui se sépare au couplage, et Y est un groupe ballast.

6. Elément d'enregistrement photographique couleur selon la revendication 5, dans lequel X représente -H, -Cl, -OCOR¹, -SAr, -SO₂R¹, -OSO₂R¹, où R¹ représente un groupe alkyle ; R² représente un groupe alkyle ou un groupe arylsulfonyle, alkoxycarbonyle, alkylsulfonamido ou carboxyle éventuellement substitué ; R³ représente un hydrogène ou un groupe alkylsulfonamido ; Ar représente un groupe aryle'; et Z représente n'importe quel groupe organique permettant de compléter le cycle.

7. Procédé de préparation d'une couche sensible au bleu dans un élément photographique photosensible aux halogénures d'argent, qui comprend la formation d'une dispersion d'un coupleur formateur de colorant d'image jaune dans un colloïde hydrophile, le mélange de la dispersion avec une émulsion aux halogénures d'argent et l'application de la composition résultante pour former une couche, procédé caractérisé en ce que le coupleur jaune est un coupleur pivalylacétanilide et le procédé comprend aussi une étape d'addition d'un polymère de polyoxyalkylène à la dispersion ou à l'émulsion, en une quantité comprise entre 0,1 et 0,6 gramme environ par gramme de coupleur jaune contenu dans la dispersion, avant de former la couche.

8. Procédé selon la revendication 7, dans lequel le polymère de polyoxyalkylène est un copolymère séquencé de polyoxyéthylène et de polyoxypropylène.

9. Procédé selon la revendication 7 ou 8, dans lequel le coupleur jaune est tel que défini dans la revendication 5 ou 6.
